

# UNITED STATES PATENT OFFICE.

JOSEF WEBER, OF ESSEN-ON-THE-RUHR, GERMANY, ASSIGNOR TO THE FIRM OF KRISTALLIT SPORTEIS-GESELLSCHAFT M. B. H., OF ESSEN-ON-THE-RUHR, GERMANY.

## IMITATION-ICE SURFACE AND PROCESS OF MAKING IT.

1,181,275.

Specification of Letters Patent.

Patented May 2, 1916.

No Drawing.

Application filed October 18, 1913. Serial No. 795,879.

To all whom it may concern:  
Be it known that I, Doctor JOSEF WEBER, residing at Salkenbergsweg 18, Essen-on-the-Ruhr, Germany, have invented certain 5 new and useful Improvements in Imitation-Ice Surface and Process of Making It, of which the following is a specification.

This invention relates to a new or improved process for the manufacture of imitation ice surfaces suitable for skating and for other sports, games or pastimes.

It has already been proposed to manufacture surfaces for skating and so on, by means of certain crystalline salts, to which latter, in some cases, other suitable substances were added. The masses thus produced however possessed rather dull surfaces and were not sufficiently smooth or glassy for skating and similar purposes. 20 Furthermore it has been suggested to moisten such surfaces with hot water and to render them smooth or slippery by brushing them mechanically. Nevertheless hitherto it has not been possible to obtain 25 a smooth or slippery surface which was the equivalent of an ice surface.

The object of the present invention is to devise a process for the manufacture of smooth or slippery and clear masses which 30 are quite similar in their appearance and qualities to ice, and therefore suited more particularly for skating.

In carrying out the invention salts of thiosulfuric acid are employed, especially 35 thiosulfate of sodium, which is liquefied by melting it in its water of crystallization and to which, preferably, borax is added. It has been found that the latter salt dissolves in the liquefied thiosulfate to a relatively 40 high degree (up to about 25 per cent.). Such addition of borax has been found to have a favorable influence upon the durability and the smoothness or slipperiness of the skating surface.

45 The process may be carried out in the following manner: Sodium thiosulfate is mixed with a certain amount of borax and this mixture is liquefied by heating. Then

this fluid mass is poured out or cast upon a suitable base, floor or surface which preferably is not perfectly smooth, but slightly roughened. The whole of the casting may be effected at one time but preferably several castings are performed if desired in such a manner as to produce superposed layers. When cooled and set, this mass has a surface which may be said to be the equivalent of an ice surface and which will not suffer damage or have its slipperiness or glassy character deteriorated by heat 60 during the summer season.

What I claim is:

1. A process for manufacturing smooth and slippery imitation ice surfaces which consists in pouring a heated mass containing sodium thiosulfate and borax upon a suitable foundation and allowing the mass to solidify.

2. A process for manufacturing smooth and slippery imitation ice surfaces, which consists in heating sodium thiosulfate mixed with borax and casting the resultant saline mass upon a suitable foundation.

3. A process for manufacturing smooth imitation ice surfaces which consists in liquefying by heating sodium thiosulfate, mixed with borax, in its crystallization water, casting the liquid saline mass upon a suitable foundation and cooling same.

4. A process for manufacturing smooth and slippery imitation ice surfaces, which consists in liquefying by heating sodium thiosulfate in its water of crystallization, dissolving borax in the resultant liquid, pouring the liquefied mass on a suitable foundation and allowing the mass to congeal by cooling.

5. An imitation ice surface, track or rink consisting of a mass containing sodium thiosulfate and borax.

In testimony whereof I affix my signature in presence of two witnesses.

JOSEF WEBER. [L.S.]

Witnesses:

ALBERT NUFER,  
JULIUS FESTNER.